

# United States Patent Office

2,964,474

Patented Dec. 13, 1960

1

2,964,474

## LUBRICATING OIL RESISTANT TO COLD SLUDGE FORMATION

Harvey E. Alford, Amherst, Ohio, assignor to The Standard Oil Company, Cleveland, Ohio, a corporation of Ohio

No Drawing. Filed Dec. 31, 1956, Ser. No. 631,512

6 Claims. (Cl. 252—18)

This invention relates to lubricating oil additives useful in the preparation of lubricating oil compositions having a lessened or substantially no tendency to form cold sludge and, more particularly, to lubricating oil compositions comprising an alkaline detergent, an antioxidant and an organic disulfide.

When an engine is operated during cold weather and in light duty "stop-and-go" operations, it rarely is heated to operating temperature for any substantial portion of the driving time. When the temperatures in the crankcase are below operating temperatures, contaminants enter the crankcase by way of blow-by. These contaminants are not dissipated because of the low operating temperatures of the oil, and have an opportunity to react or to catalyze reactions in the oil. These reactions result in the formation of what is called cold sludge, a black, mayonnaise-like substance. One of the most important problems today is how to combat cold sludge, because most cars used in city driving are subjected to this type of driving conditions during cold weather.

It has now been determined that when oil containing an alkaline sulfonate type detergent, and a thiophosphate type antioxidant as additives has added thereto an organic disulfide, the oil does not develop cold sludge when the engine is operated at low temperatures for long periods of time. It is thought that this combination of additives is effective because it destroys the contaminants which enter the oil. These contaminants are thought to include organic peroxides and hydroperoxides. The peroxides are capable of catalyzing reactions that lead to the formation of high polymers, and it is believed that high polymers are major components of cold sludge. Accordingly, the effectiveness of the additive of the invention is thought to depend upon its ability to react with peroxides to destroy them, and the additive has been evaluated on the basis of a screening test determining decomposition of cumene hydroperoxide at 100° F.

The alkaline sulfonate type detergent and the thiophosphate type antioxidants are well known in the lubricating oil additive art. The preferred alkaline sulfonate type detergent is formed from barium octadecylsulfonate and barium carbonate. This additive is well known and needs no further description. The barium carbonate is thought to neutralize the acids that are formed. The preferred antioxidant is zinc octyl dithiophosphate which has a molecular weight of about 321.4 and has the formula  $ZnC_8H_{17}PS(S)_2$ . It is the zinc salt of a phosphorus pentasulfide-octyl mercaptan reaction product. The zinc octyldithiophosphate is an antioxidant and, in addition, inhibits corrosion and wear.

The organic disulfide has the general formula RSSR, where R is a hydrocarbon radical having from 3 to 18 carbon atoms, preferably from 3 to 8 carbon atoms, and can be aliphatic, aryl, alkaryl, and aralkyl; for example, propyl, butyl, hexyl, octyl, decyl, dodecyl, tetradecyl, hexadecyl and octadecyl; phenyl, benzyl, methylbenzyl, methylphenyl, xylyl, naphthyl, octylphenyl, nonylphenyl, dodecylphenyl, trimethylbenzyl, methyethylbenzyl and

2

propylbenzyl. These are known compounds, readily prepared by conventional procedures using sodium disulfide and the corresponding chlorinated hydrocarbon, the chlorine being affixed to the carbon atom which is to be attached to the disulfide chain.

Very small amounts of the additives of the invention will give a marked improvement in lessening the formation of cold sludge. As little as 1.0% of the total mixture of additives is effective, and amounts between 2% and 10% are preferred. Use of amounts in excess of 20% usually cannot be justified economically. Of the total mixture of additives, the disulfide is present in an amount within the range from 8 to 70 parts by weight (p.b.w.). The other three ingredients are combined and are present in an amount of 35 to 135 p.b.w. In this combination, the barium octadecyl sulfonate is present in an amount within the range from 20 to 60 p.b.w., the barium carbonate in an amount within the range from 10 to 30 p.b.w., and the zinc octyl dithiophosphate in an amount within the range from 15 to 45 p.b.w.

The additives of the invention can be used to improve the cold sludge characteristics of any petroleum hydrocarbon oil of lubricating viscosity. The S.A.E. viscosities for lubricating oils range from No. 10 to No. 70. Oils having S.A.E. Nos. 10 to 40 have a viscosity within the range from 90 to 255 SSU at 130° F., and those oils having S.A.E. Nos. 40 to 70 have a viscosity within the range from 80 to 150 SSU at 210° F. The acid-treated and solvent-extracted oils are equally useful in the compositions of the invention. The oils can be blended from finished neutral oils of light and heavy viscosities and can include suitable bright stocks. It can also include other conventional additives such as V.I. improvers. It is impossible here to give a complete description of the various methods used in the preparation of lubricating oils, but reference is made to the text by Georgi, entitled Motor Oils and Engine Lubrication, published by Reinhold Publishing Corporation, New York (1950), chapter V, wherein the various types of lubricating oils are discussed fully. Any of the oils mentioned therein can be employed in the composition of the invention.

The composition of the invention is prepared simply by mixing the additives, either singly or together, with the oil, at room temperature. The additives are soluble or dispersible in the oil, and disperse therein instantaneously. No solvents are required but the additives can be placed in solution in a hydrocarbon.

The following examples represent, in the opinion of the inventor, the best embodiment of his invention.

In the examples, the effectiveness of the additive to decompose peroxides was determined by a screening test involving decomposition of cumene hydroperoxide at 100° F. Fifty (50) grams of a cetane or solvent-extracted neutral oil (140 SSU at 210° F.) was used as the solvent. One solution was made by adding 2.25% of a mixture comprising 40 p.b.w. barium octadecylsulfonate, 20 p.b.w. barium carbonate, and 28 p.b.w. zincoctyldithiophosphate. Another solution was made by adding the disulfide in a concentration of 0.1 equivalent per equivalent of peroxide. A third solution contained both. All were heated at 280° F. for four hours while air was passed through at a rate of 35 liters per hour. To each solution was then added 5% of cumene hydroperoxide, and the solutions were heated for two hours at 100° F. The amount of peroxide decomposed was then determined.

The method used to analyze peroxides is described in Industrial and Engineering Chemistry, Analytical Edition, 19, 976 (1947). A 5 ml. sample was taken and weighed. To this was added 40 cc. of isopropanol and 2 cc. of glacial acetic acid. The mixture was heated to reflux, and 10 cc. of saturated sodium iodide solution was added. Thereafter, the mixture was refluxed for five minutes, 5

cc. of distilled water was added, and the mixture titrated was 0.1 n sodium thiosulfate.

## EXAMPLES 1 AND 2

A solution was prepared containing 2.25% by weight of a mixture of 40 p.b.w. barium octadecylsulfonate, molecular weight 783.4, formula  $\text{Ba}(\text{SO}_3\text{C}_{18}\text{H}_{27})_2$ , 20 p.b.w. barium carbonate, and 28 p.b.w. zinc octyldithiophosphate  $\text{ZnC}_8\text{H}_{17}\text{PS}(\text{S})_2$ , molecular weight 321.4, in solvent-extracted neutral oil, 140 SSU at 210° F. Separate additional solutions were prepared of 0.58% di-n-butyl-disulfide (0.1 equivalent) and 0.8% dibenzyl-disulfide (0.1 equivalent) using this solvent-extracted neutral oil alone, and the same oil containing the sulfide and the barium octadecylsulfonate, barium carbonate and zinc octyldithiophosphate. All of these solutions then were tested by the screening test described above, after heat treatment for four hours at 280° F. with air-blowing at 35 liters per hour. The results were as follows:

Table I

| Example No. | Compound                                                                                                             | Percent   | Relative Amounts of Peroxide Decomposed |
|-------------|----------------------------------------------------------------------------------------------------------------------|-----------|-----------------------------------------|
| Control     | Mixture of 40 p.b.w. Barium Octadecylsulfonate, 20 p.b.w. Barium Carbonate, and 28 p.b.w. Zinc Octyldithiophosphate. | 2.25      | 100                                     |
| 1a          | Di-n-butyl-disulfide only                                                                                            | 0.58      | 12.7                                    |
| b           | Control+di-n-butyl-disulfide                                                                                         | 2.25+0.58 | 143                                     |
| 2a          | Dibenzyl disulfide only                                                                                              | 0.8       | 11.0                                    |
| b           | Control+dibenzyl disulfide                                                                                           | 2.25+0.8  | 140                                     |

A comparison of the results for Examples 1 and 2 with the control shows that the two groups of additives together are far superior to either alone. The combination of additives in accordance with the invention gives a synergistic effect on the decomposition of cumene hydroperoxide.

## EXAMPLE 3

The above tests were repeated, this time employing compositions in which the additives were dissolved in cetane rather than in the solvent-extracted neutral oil, and the additives were not subjected to a prior heat treatment before testing. The results obtained were as follows:

Table II

| Example No. | Compound                                                                                                             | Percent           | Relative Amounts of Peroxide Decomposed |
|-------------|----------------------------------------------------------------------------------------------------------------------|-------------------|-----------------------------------------|
| Control     | Mixture of 40 p.b.w. Barium Octadecylsulfonate, 20 p.b.w. Barium Carbonate, and 28 p.b.w. Zinc Octyldithiophosphate. | 2.25              | 100                                     |
| 3           | {Di-n-butyl-disulfide<br>Control+di-n-butyl disulfide}                                                               | 0.58<br>2.25+0.58 | 12.7<br>128                             |

Once again, the mixture of additives of the invention is far superior.

In order to determine the effect of the additives of the invention on the formation of cold sludge in an automobile engine, engine tests were conducted on oils of the composition hereinafter indicated. The tests were conducted in a single-cylinder ethyl engine under the following conditions:

Table III

| Time (Hrs.) | R.P.M.         | Oil Temperature, ° F. | Jacket Temperature, ° F. | AFR                 |
|-------------|----------------|-----------------------|--------------------------|---------------------|
| 5           |                |                       |                          |                     |
| 2           | 1,280<br>1,280 | 100±5<br>300±5        | 100±5<br>210+2, -5       | Approx. 9:1<br>13:1 |

Test Duration: 15 cycles, 60 hours.  
Oil Charge: 2,000 cc.

The effect of the additives in the engine was determined by the amount of pentane insolubles that were formed in the oil. The result of the tests are shown in the following table:

Table IV

ETHYL ENGINE TEST RESULTS

| Compound                                                                                                                                                             | Heat-Treat <sup>1</sup> | Percent Pentane Insolubles |
|----------------------------------------------------------------------------------------------------------------------------------------------------------------------|-------------------------|----------------------------|
| 2.25% of a mixture of 40 p.b.w. Barium Octadecylsulfonate, 20 p.b.w. Barium Carbonate, and 28 p.b.w. Zinc Octyldithiophosphate.                                      | No-----                 | 1.80                       |
| 1.16% (0.2 eq.) Di-n-butyl-disulfide+2.25% of a mixture of 40 p.b.w. Barium Octadecylsulfonate, 20 p.b.w. Barium Carbonate, and 28 p.b.w. Zinc Octyldithiophosphate. | Yes-----                | 0.87                       |
| 1.16% (0.2 eq.) Di-n-Butyl-disulfide+2.25% of a mixture of 40 p.b.w. Barium Octadecylsulfonate, 20 p.b.w. Barium Carbonate, and 28 p.b.w. Zinc Octyldithiophosphate. | No-----                 | 0.829                      |

<sup>1</sup> 4 hours at 280° F. with air-blowing at 35 liters per hour.

It is evident that the combination of additives in accordance with the invention is far superior to either alone, in that much less pentane insolubles are formed in the oil. Heat treatment of the additive mixture prior to use is not significant.

I claim:

1. An additive for a mineral lubricating oil for the lessening of cold sludge formation in operation of a lubricating oil at low temperatures, consisting essentially of 20 to 60 parts by weight barium octadecyl sulfonate, from 10 to 30 parts by weight barium carbonate, from 15 to 45 parts by weight zinc octyl dithiophosphate, and from 8 to 70 parts by weight of an organic disulfide having the formula  $\text{RSSR}$ , where  $\text{R}$  is a hydrocarbon group having from 3 to 18 carbon atoms.

2. An additive in accordance with claim 1, in which the organic disulfide is di-n-butyl-disulfide.

3. An additive in accordance with claim 1, in which the organic disulfide is dibenzyl disulfide.

4. A mineral lubricating oil composition consisting essentially of a mineral lubricating oil and an amount of an additive in accordance with claim 1 within the range from 1% to 20% sufficient to lessen cold sludge formation during operation of the oil at low temperatures.

5. A mineral lubricating oil composition in accordance with claim 4, in which the organic disulfide is di-n-butyl-disulfide.

6. A mineral lubricating oil composition in accordance with claim 4, in which the organic disulfide is dibenzyl disulfide.

## References Cited in the file of this patent

## UNITED STATES PATENTS

|    |           |                        |               |
|----|-----------|------------------------|---------------|
| 65 | 2,110,281 | Adams et al. -----     | Mar. 8, 1938  |
|    | 2,257,890 | Sloane -----           | Oct. 7, 1941  |
|    | 2,369,632 | Cook et al. -----      | Feb. 13, 1945 |
|    | 2,398,415 | Denison et al. -----   | Apr. 16, 1946 |
|    | 2,398,416 | Denison -----          | Apr. 16, 1946 |
| 70 | 2,451,345 | McNab -----            | Oct. 12, 1948 |
|    | 2,501,731 | Mertes -----           | Mar. 28, 1950 |
|    | 2,676,925 | Lindstrom et al. ----- | Apr. 27, 1954 |